

1

3,594,291

## BRIGHT ZINC PLATING FROM AN ACID ELECTROLYTE

Hans-Gunther Todt and Günter Voss, Berlin, Germany, assignors to Schering AG, Berlin, Germany  
No Drawing. Filed July 24, 1969, Ser. No. 844,644  
Claims priority, application Germany, Aug. 10, 1968,  
P 17 17 983.4  
Int. Cl. C23b 5/12, 5/46

U.S. CL. 204—55

8 Claims

### ABSTRACT OF THE DISCLOSURE

Mirror bright zinc electrodeposits are formed from acid zinc plating solutions containing as brighteners N-polyvinylpyrrolidone-(2) and a ketone of the formula



wherein  $R_1$  is phenyl, mono- or dihydroxyphenyl or trihydroxyphenyl methylenedioxyphenyl, mono-, di- or tri-lower-alkylphenyl, mono- or di- or tri-lower-alkoxyphenyl, furyl, thieryl, coumaryl, or pyridyl, and  $R_2$  may be lower alkyl, lower alkenyl, lower-alkyl-carbonyl-lower-alkylene, cyano-lower-alkylene, lower-alkoxy-carbonyl-lower-alkylene, or  $-(CH=CH)_n-C_6H_5$ ,  $n$  being 1 or 0.

This invention relates to the electrodeposition of bright zinc, and particularly to bright zinc plating from acid electrolytes.

A wide variety of bright zinc plating solutions of the cyanide type is available. The cyanide baths are relatively unstable because of the decomposition of cyanide to carbonate, and the cyanide drag-out into rinsing baths presents a serious disposal problem. The deposits formed from known acid zinc plating baths free from organic complexing agents are at best smooth, but not bright, and complex forming organic components in acid zinc plating solutions, such as EDTA present a disposal and pollution problem as difficult to solve as that caused by cyanide. Zinc and other heavy metals cannot be precipitated from the rinse water and other wastes bearing EDTA by means of alkaline reagents. Bright coatings can be produced from baths containing EDTA (ethylenediaminetetra-acetic acid) only if other heavy metals, particularly iron, copper, and nickel, are carefully and initially removed.

The object of the invention is the provision of a brightener system for acid zinc plating solutions which permits the zinc dragged out into rinsing baths to be precipitated by an alkaline reagent because of the absence of complex forming compounds, is insensitive to substantial amounts of other heavy metal, provides bright and ductile deposits over a wide range of cathode current densities, and is stable under the operating conditions usual for the electrodeposition of dull coatings from acid electrolytes including agitation by means of compressed air.

Such a brightener system has been found in the combination of N-polyvinylpyrrolidone-(2) with a secondary brightener of the formula



wherein  $R_1$  is



3



4



5

10

15

20

25

30

35

40

45

50

55

60

65

70

75

80

85

90

95

100

105

110

115

120

125

130

135

140

145

150

155

160

165

170

175

180

185

190

195

200

205

210

215

220

225

230

235

240

245

250

255

260

265

270

275

280

285

290

295

300

305

310

315

320

325

330

335

340

345

350

355

360

365

370

375

380

385

390

395

400

405

410

415

420

425

430

435

440

445

450

455

460

465

470

475

480

485

490

495

500

505

510

515

520

525

530

535

540

545

550

555

560

565

570

575

580

585

590

595

600

605

610

615

620

625

630

635

640

645

650

655

660

665

670

675

680

685

690

695

700

705

710

715

720

725

730

735

740

745

750

755

760

765

770

775

780

785

790

795

800

805

810

815

820

825

830

835

840

845

850

855

860

865

870

875

880

885

890

895

900

905

910

915

920

925

930

935

940

945

950

955

960

965

970

975

980

985

990

995

1000

1005

1010

1015

1020

1025

1030

1035

1040

1045

1050

1055

1060

1065

1070

1075

1080

1085

1090

1095

1100

1105

1110

1115

1120

1125

1130

1135

1140

1145

1150

1155

1160

1165

1170

1175

1180

1185

1190

1195

1200

1205

1210

1215

1220

1225

1230

1235

1240

1245

1250

1255

1260

1265

1270

1275

1280

1285

1290

1295

1300

1305

1310

1315

1320

1325

1330

1335

1340

1345

1350

1355

1360

1365

1370

1375

1380

1385

1390

1395

1400

1405

1410

1415

1420

1425

1430

1435

1440

1445

1450

1455

5

## EXAMPLE 2

Zinc sulfate ( $ZnSO_4 \cdot 7H_2O$ ): 290 g./l.  
 Ammonium chloride: 25 g./l.  
 Polyvinylpyrrolidone-(2): 5 g./l.  
 Propiophenone: 0.1 g./l.  
 Nonylphenol-ethyleneoxide addition compound: 0.04 g./l.  
 pH: 4.5  
 Temperature: 30° C.  
 Current density: 0.1-6.0 amps/dm.<sup>2</sup>  
 Cathode rod agitation

## EXAMPLE 3

Zinc chloride ( $ZnCl_2$ ): 70 g./l.  
 Ammonium sulfate: 130 g./l.  
 Sodium chloride: 10 g./l.  
 Polyvinylpyrrolidone-(2): 3 g./l.  
 Benzalacetone: 0.1 g./l.  
 Ethyl benzoylacetate: 0.1 g./l.  
 Sodium ethylhexylsulfate: 0.5 g./l.  
 pH: 5.0  
 Temperature: 25° C.  
 Current density: 0.1-5.0 amps/dm.<sup>2</sup>  
 Air agitation

## EXAMPLE 4

Zinc sulfate ( $ZnSO_4 \cdot 7H_2O$ ): 145 g./l.  
 Ammonium chloride: 53 g./l.  
 Boric acid: 20 g./l.  
 Polyvinylpyrrolidone-(2): 3 g./l.  
 1-(2-Furyl)-1'-buten-3-one: 0.1 g./l.  
 Nonylphenol-ethyleneoxide: 0.4 g./l.  
 pH: 4.2  
 Temperature: 25° C.  
 Current density: 0.1-5 amps/dm.<sup>2</sup>  
 Cathode rod agitation

## EXAMPLE 5

Zinc sulfate ( $ZnSO_4 \cdot 7H_2O$ ): 290 g./l.  
 Ammonium chloride: 25 g./l.  
 Polyvinylpyrrolidone-(2): 5 g./l.  
 3-Acetylpyridine: 3 g./l.  
 Fatty alcohol polyglycoether: 0.2 g./l.  
 pH: 4.8  
 Temperature: 30° C.  
 Current density: 0.1-7.5 A./dm.<sup>2</sup>  
 Cathode rod agitation

## EXAMPLE 6

Zinc sulfate ( $ZnSO_4 \cdot 7H_2O$ ): 145 g./l.  
 Ammonium chloride: 53 g./l.  
 Polyvinylpyrrolidone-(2): 2.5 g./l.  
 1-(2-Furyl)-1'-buten-3-one: 0.2 g./l.  
 Sodium dodecylphenol-polyglycol-ether-sulfate: 0.1 g./l.  
 pH: 5.0  
 Temperature: 25° C.  
 Current density: 0.1-5 amps/dm.<sup>2</sup>  
 Cathode rod agitation

## EXAMPLE 7

Zincsulfate ( $ZnSO_4 \cdot 7H_2O$ ): 145 g./l.  
 Ammoniumchloride: 53 g./l.  
 Boric acid: 20 g./l.  
 Polyvinylpyrrolidone-(2): 3 g./l.  
 3-methoxy-benzaleacetone: 0.15 g./l.  
 pH: 5.5  
 Temperature: 25° C.  
 Current density: 0.1-5.0 A./dm.<sup>2</sup>  
 Air agitation

## EXAMPLE 8

Zinc sulfate ( $ZnSO_4 \cdot 7H_2O$ ): 290 g./l.  
 Ammoniumchloride: 25 g./l.

6

Polyvinylpyrrolidone-(2): 5 g./l.  
 4-methoxy-benzylideneacetone: 0.05 g./l.  
 Nonylphenol-ethyleneoxide addition compound: 0.04 g./l.  
 pH: 4.5  
 5 Temperature: 30° C.  
 Current density: 0.1-6 amps/dm.<sup>2</sup>  
 Cathode rod agitation

## EXAMPLE 9

10 Zinc chloride ( $ZnCl_2$ ): 70 g./l.  
 Ammonium sulfate: 130 g./l.  
 Sodiumchloride: 10 g./l.  
 Polyvinylpyrrolidone-(2): 3 g./l.  
 Piperonylideneacetylacetone: 0.2 g./l.  
 15 Sodium ethylhexylsulfate: 0.5 g./l.  
 pH: 5.0  
 Temperature: 25° C.  
 Current density: 0.1-5 amps/dm.<sup>2</sup>  
 Air agitation

20 EXAMPLE 10

Zinc sulfate ( $ZnSO_4 \cdot 7H_2O$ ): 145 g./l.  
 Ammoniumchloride: 53 g./l.  
 Boric acid: 20 g./l.  
 Polyvinylpyrrolidone-(2): 3 g./l.  
 25 Piperonylidenebenzylacetone: 0.1 g./l.  
 Nonylphenol-ethyleneoxide: 0.4 g./l.  
 pH: 4.2  
 Temperature: 25° C.  
 Current density: 0.1-5 amps/dm.<sup>2</sup>  
 30 Cathode rod agitation

## EXAMPLE 11

Zinc sulfate ( $ZnSO_4 \cdot 7H_2O$ ): 145 g./l.  
 35 Ammoniumchloride: 53 g./l.  
 Polyvinylpyrrolidone-(2): 2.5 g./l.  
 2-thienylideneaceton: 0.2 g./l.  
 Sodium dodecylphenol-polyglycoether-sulfate: 0.25 g./l.  
 pH: 4.8  
 40 Temperature: 30° C.  
 Current density: 0.1-5 amps/dm.<sup>2</sup>  
 Cathode rod agitation

## EXAMPLE 12

45 Zinc sulfate ( $ZnSO_4 \cdot 7H_2O$ ): 290 g./l.  
 Ammoniumchloride: 25 g./l.  
 Polyvinylpyrrolidone-(2): 5 g./l.  
 A-acetylcoumarin: 0.4 g./l.  
 pH: 4.8  
 50 Temperature: 30° C.  
 Current density: 0.1-5 amps/dm.<sup>2</sup>  
 Cathode rod agitation  
 What is claimed is:  
 1. In an aqueous acid plating electrolyte for the deposition of zinc electrodeposits in the absence of organic compounds forming complex ions with heavy metals, the electrolyte containing a source of zinc ions, the improvement which comprises having present in said electrolyte:  
 55 (a) 0.5 to 100 grams per liter N-polyvinylpyrrolidone-(2) dispersed in said electrolyte as a primary brightener; and  
 (b) .01 to 0.5 gram per liter of a secondary brightener dispersed in said electrolyte, said secondary brightener being a compound of the formula



wherein  $R_1$  is



75  $R_2$  is lower alkyl, lower alkenyl, lower alkyl-carbonyl-

lower-alkylene, cyano-lower alkylene, lower-alkoxy-carbonyl-lower-alkylene, or



$R_3$ ,  $R_4$  and  $R_5$  each are hydrogen, hydroxy, lower alkyl, or lower alkoxy, and  $R_3$  and  $R_4$  together represent the methylenedioxy group, and  $n$  is 1 or 0.

2. In an electrolyte as set forth in claim 1, the concentration of said N-polyvinylpyrrolidone-(2) being between 2 and 10 grams per liter, and the concentration of said secondary brighteners between 0.05 and 0.3 gram per liter.

3. In an electrolyte as set forth in claim 1,  $R_2$  being methyl or ethyl.

4. In an electrolyte as set forth in claim 3,  $R_2$  being ethenyl.

5. In an electrolyte as set forth in claim 1,  $R_2$  being  $-\text{CH}_2\text{COCH}_3$ .

6. In an electrolyte as set forth in claim 1,  $R_2$  being



7. In an electrolyte as set forth in claim 1, the pH being 3 to 6.

10 8. A method of forming bright zinc electrodeposits which comprises making an object the cathode in the electrolyte as set forth in claim 1.

#### References Cited

##### UNITED STATES PATENTS

- |    |           |         |                       |         |
|----|-----------|---------|-----------------------|---------|
| 15 | 2,853,444 | 9/1958  | Pye et al. -----      | 204—55X |
|    | 3,005,759 | 10/1961 | Safranek et al. ----- | 204—55  |
|    | 3,285,840 | 11/1966 | Lindemann -----       | 204—55  |

GERALD L. KAPLAN, Primary Examiner